

# United States Patent [19]

Dudek et al.

[11] 3,907,555

[45] Sept. 23, 1975

[54] NICKEL ALLOYS

[75] Inventors: **Ronald P. Dudek**, River Grove; **Peter Kosmos**, Alsip; **John A. Tesk**, Wood-Ridge, all of Ill.

[73] Assignee: **Howmedica, Inc.**, Chicago, Ill.

[22] Filed: **Sept. 26, 1974**

[21] Appl. No.: **509,557**

**Related U.S. Application Data**

[63] Continuation-in-part of Ser. No. 317,594, Dec. 22, 1972, Pat. No. 3,841,868.

[52] **U.S. Cl.** ..... 75/171

[51] **Int. Cl.<sup>2</sup>** ..... **C22C 19/05**

[58] **Field of Search** ..... 75/171, 170; 148/32, 32.5

[56] **References Cited**

UNITED STATES PATENTS

|           |         |              |        |
|-----------|---------|--------------|--------|
| 2,226,079 | 12/1940 | Spanner..... | 75/172 |
| 2,460,595 | 2/1949  | Reich.....   | 75/134 |
| 3,134,671 | 5/1964  | Prosen.....  | 75/172 |

|           |        |                     |        |
|-----------|--------|---------------------|--------|
| 3,340,050 | 9/1967 | Nielsen et al. .... | 75/165 |
| 3,554,738 | 1/1971 | Beldham et al. .... | 75/134 |
| 3,574,610 | 4/1971 | Prosen .....        | 75/165 |
| 3,574,611 | 4/1971 | Prosen .....        | 75/165 |
| 3,679,402 | 7/1972 | Hirschhorn .....    | 75/165 |

*Primary Examiner*—R. Dean  
*Attorney, Agent, or Firm*—Pennie & Edmonds

[57] **ABSTRACT**

A corrosion resistant precision casting alloy particularly suitable for use as a dental alloy comprises essentially, by weight, at least 60 percent nickel, 10 to 25 percent chromium, up to 10 percent molybdenum, 0.50 to 1.5 percent manganese, up to 6.5 percent tin, 1.0 to 7.5 percent gallium, up to 5 percent copper, up to 4 percent silicon, up to 2.0 percent aluminum, up to 5 percent cobalt and up to 0.2 percent carbon, the combined total amount of tin and gallium not exceeding 7.5 percent.

**7 Claims, No Drawings**

## NICKEL ALLOYS

## RELATED APPLICATION

This application is a continuation-in-part of applicants' copending application Ser. No. 317,594, filed Dec. 22, 1972 entitled "Nickel Alloy," now U.S. Pat. No. 3,841,868.

## BACKGROUND OF THE INVENTION

## 1. Field of the Invention

This invention relates to corrosion resistant precision casting alloys particularly suitable for use as dental alloys.

## 2. Prior Art

Metals and metal alloys are used extensively in restorative and corrective dentistry for removable restorations, inlays, crowns, and bridges, orthodontic appliances, and the like. Dental alloys must meet stringent physical and chemical requirements. First, the chemical nature of the alloy must be such that no harmful physiological effects are produced on the patient or the operator. The alloy must be stainless and resistant to attack by the various acid and alkaline substances naturally present in the mouth and in foods and beverages. It must be capable of being fabricated into the desired dental appliances by dentists and technicians and yet must be hard enough and strong enough to resist wear and deformation in use, and it must be capable of being cast to form precision castings free of inclusions, blow holes and other defects.

Gold alloys were originally the most widely used and useful of the dental alloys. However, the high cost and scarcity of gold led to the development of dental alloys comprising predominantly cobalt and chromium with minor amounts of tungsten, nickel and other metals. These cobalt-chromium base dental alloys are exemplified by those disclosed in U.S. Pat. Nos. 1,961,626 and 2,134,423 to Enrique G. Touceda. More recent work has led to the development of dental alloys comprising predominantly nickel and chromium with minor amounts of molybdenum, iron, copper and other metals. These newer nickel-chromium base dental alloys are exemplified by the alloy disclosed in U.S. Pat. No. 2,597,495 to Jackson and Simmons. All of these prior dental alloys possess to a greater or lesser extent the characteristics required of such alloys as previously discussed. However, none possesses all of the required characteristics to the optimum extent, and research and development of new dental alloys with improved characteristics is constantly taking place.

In our copending application Ser. No. 317,594 we have described an improved corrosion resistant alloy that comprises essentially, by weight, 15.0 to 25 percent chromium, 3.0 to 6.0 percent molybdenum, 1.0 to 4.0 percent tin, 0.5 to 1.5 percent manganese, 0.5 to 5.0 percent copper, 1.0 to 4.0 percent silicon, up to 1.0 percent aluminum, up to 1.0 percent cobalt, up to 0.2 percent carbon and the balance (52.3 to 79.0 percent) nickel. The resulting alloy is capable of being cast to form precision castings that are free of inclusion, blow holes and other defects, and the alloy is relatively easy to work while possessing adequate strength and hardness.

The aforesaid alloy contains a small but significant amount of tin which greatly improves the fluidity of the molten alloy and also contributes to the strength and hardness of the cast alloy without unduly reducing the

elongation of the alloy. As a result of further investigations with respect to this and related alloys we have found that gallium imparts essentially the same characteristics to the molten and cast alloy as tin and may be included in the alloy along with tin or in place of tin to obtain an alloy having excellent casting properties and that is relatively easy to work while possessing adequate strength and hardness. In addition, we have found that the amount of tin and/or gallium included in the alloy may be significantly increased over the amount employed in the alloy of our copending application and further that the alloy can optionally contain significant amounts of copper, silicon, aluminum and cobalt.

## SUMMARY OF THE INVENTION

The improved corrosion resistant alloy of the invention comprises essentially, by weight, at least 60% nickel, 10 to 25% chromium, up to 10% molybdenum, 20 0.50 to 1.50% manganese, up to 6.5% tin, 1.0 to 7.5% gallium, up to 5% copper, up to 4.0% silicon, up to 2.0% aluminum, up to 5% cobalt and up to 0.2% carbon, the combined total amount of tin and gallium not exceeding 7.5%. The resulting alloy is capable of being cast to form precision castings that are free of inclusions, blow holes and other defects, and the alloy is relatively easy to work while possessing adequate strength and hardness.

## 30 DESCRIPTION OF PREFERRED EMBODIMENT

The corrosion resistant alloy of our invention consists predominantly of nickel and chromium with minor but significant amounts of other metals that modify the physical properties (for example, its fusion point, hardness and workability) of the basic alloy composition. In general, the proportion of nickel to chromium in the basic alloy composition may range from about 2:1 to about 5:1, and in the preferred composition is about 3.5:1. Nickel is the major component of the alloy and is employed for its inherent resistance to corrosion. Chromium, the other predominant component of the basic alloy composition, enhances the corrosion resistance of the alloy and also is a solid solution/precipitation hardener. In addition, a small but significant amount of manganese acts as a safeguard against possible sulfur contamination and a small amount of molybdenum is advantageously employed to enhance the corrosion resistance of the alloy and as a powerful solid solution/precipitation hardener. Optionally, the alloy may contain a small amount of silicon that acts as a de-oxidizer and also lowers the fusion temperature of the alloy, and a small amount of copper may be added to improve the surface finish of the cast alloy. Small amounts of cobalt and aluminum, the latter as a deoxidizer and precipitation hardener, and a very small amount of carbon may also be present in the alloy. Lastly, the alloy of the invention contains a small but significant amount of gallium with or without a small amount of tin which greatly improves the fluidity of the molten alloy and also contributes to the strength and hardness of the cast alloy without unduly reducing the elongation of the alloy.

As previously noted, we have found that gallium imparts essentially the same characteristics to the molten and cast alloy as is imparted to the alloy by tin, and further that gallium may be included in the alloy along with tin or in place of tin to obtain an alloy having ex-

cellent casting properties and that is relatively easy to work while possessing adequate strength and hardness. In addition we have found that the amount of tin and gallium included in the alloy may be significantly increased over the amount employed in the alloy of our copending application Ser. No. 317,594, and further that the alloy can optionally contain significant amounts of copper, silicon, aluminum, cobalt and molybdenum, as hereinafter described.

The relative proportions of the various elements comprising the new alloy composition has been determined as the result of an intensive investigation to obtain an alloy having optimum chemical and physical properties. Specifically, we have found that the alloy composition of the invention should contain at least 60 percent by weight nickel, from 10 to 25 percent by weight chromium, up to 10 percent by weight molybdenum, from 0.50 to 1.5 percent by weight manganese, from 1.0 to 7.5 percent by weight gallium, up to 6.5 percent by weight tin, up to 5 percent by weight copper, up to 4.0 percent silicon, up to 2.0 percent by weight aluminum, up to 5 percent by weight cobalt and up to 0.2 percent by weight carbon. The combined total amount of gallium and tin should not exceed about 7.5 percent by weight of the composition. Moreover, it should be noted that molybdenum, tin, copper, silicon, aluminum, cobalt, and carbon are optional constituents of the alloy composition, and further that gallium is an essential constituent thereof. A corrosion resistant alloy which contains the aforementioned components in the amounts specified may be readily cast to produce precision castings that may be easily finished and that have the necessary strength and hardness for the applications intended. In particular, the presence of gallium and tin in the alloy composition effects a significant improvement in these essential characteristics.

The following specific examples describe the preparation of preferred alloy compositions of the invention.

#### EXAMPLE I

A base alloy composition comprising 68.25 parts by weight nickel, 20.0 parts by weight chromium, 4.5 parts by weight molybdenum and 1.25 parts by weight manganese was prepared by melting the substantially pure components in a crucible 1.5 parts by weight copper, 2.5 parts by weight silicon and, most important, 2.0 parts by weight tin were then added to the alloy melt. After the molten ingredients were thoroughly mixed to form a homogenous melt, the molten alloy was cast into a mold or investment of refractory material to obtain a cast metal shape. Several such investment castings were made. In each case the resulting cast metal shape conformed precisely to the shape of the investment mold and was without blow holes, inclusions or other defects. The alloy shape that was allowed to air-cool in its investment mold had a Rockwell B hardness of 83, and 0.2 percent yield strength of 49,500 psi and a maximum elongation of 13 percent. When cooling was accelerated by the water quenching of the alloy shape - investment mold composite, the alloy had a Rockwell B hardness of 82, and 0.2 percent yield strength of 42,500 psi and a maximum elongation of 17 percent. Further reductions in the Rockwell B hardness and the 0.2 percent yield strength to values of 80 and 42,000 psi respectively accompanied by an increase in the maximum elongation to 25 percent were accomplished by annealing of the alloy shape at 2000°F. for 30 min-

utes after which the alloy was quenched in water. The generally good working characteristics typical of the alloy when air cooled can therefore be improved by the two aforementioned techniques or similar treatments following casting. All of these physical characteristics reflect a substantial improvement over the properties of similar, but tin-free, corrosion resistant precision casting alloys known in the prior art.

#### EXAMPLE II

The alloy composition of Example I was modified by the substitution of 1 percent by weight of gallium for 1 percent by weight of tin (one half of the tin) in the composition to obtain a corrosionresistant dental alloy having the composition listed below. The molten alloy was cast into investment cast shapes to provide test specimens free from defects and having the physical characteristics also listed below

##### Composition (% by weight) and properties

|                                 |       |    |        |
|---------------------------------|-------|----|--------|
| Ni                              | 68.25 | Si | 2.50   |
| Cr                              | 20.00 | Cu | 1.50   |
| Mo                              | 4.50  | Sn | 1.00   |
| Mn                              | 1.25  | Ga | 1.00   |
| Proportional limit (psi)        |       |    | 31,600 |
| 0.2% Yield Strength (psi)       |       |    | 42,600 |
| Ultimate Tensile Strength (psi) |       |    | 66,300 |
| Elongation (%)                  |       |    | 11     |
| Rockwell "B" Hardness           |       |    | 82     |

#### EXAMPLE III

The alloy composition of Example I was modified by the substitution of 2 percent by weight of gallium for the 2 percent by weight of tin present in the alloy to obtain a corrosion resistant dental alloy having the composition listed below. The molten alloy was cast into investment cast shapes to provide test specimens free from defects and having the physical characteristics also listed below.

##### Composition (% by weight) and properties

|                                 |       |    |        |
|---------------------------------|-------|----|--------|
| Ni                              | 68.25 | Si | 2.50   |
| Cr                              | 20.00 | Cu | 1.50   |
| Mo                              | 4.50  | Ga | 2.00   |
| Mn                              | 1.25  |    |        |
| Proportional limit (psi)        |       |    | 44,700 |
| 0.2% Yield Strength (psi)       |       |    | 51,500 |
| Ultimate Tensile Strength (psi) |       |    | 79,000 |
| Elongation (%)                  |       |    | 14     |
| Rockwell "B" Hardness           |       |    | 81     |

#### EXAMPLE IV

An alloy having the composition listed below was prepared in accordance with the procedure described in the Example I, and test specimens were prepared by investment casting of the alloy to obtain defect-free cast alloy shapes having the physical characteristics also listed below.

##### Composition (5% by weight) and properties

|    |       |    |     |
|----|-------|----|-----|
| Ni | 66.25 | Si | 2.5 |
| Cr | 20.00 | Cu | 1.5 |

-Continued

| Composition (% by weight) and properties |        |    |     |
|------------------------------------------|--------|----|-----|
| Mo                                       | 4.50   | Sn | 3.0 |
| Mn                                       | 1.25   | Ga | 1.0 |
| Proportional Limit (psi)                 | 38,600 |    |     |
| 0.2% Yield Strength (psi)                | 47,500 |    |     |
| Ultimate Tensile Strength (psi)          | 69,800 |    |     |
| Elongation (%)                           | 6      |    |     |
| Rockwell "B" Hardness                    | 87     |    |     |

10

## EXAMPLE V

An alloy having the composition listed below was prepared in accordance with the procedure described in the Example I, and test specimens were prepared by investment casting of the alloy to obtain defect-free cast alloy shapes having the physical characteristics also listed below.

| Composition (% by weight) and properties |        |    |     |
|------------------------------------------|--------|----|-----|
| Ni                                       | 66.25  | Si | 2.5 |
| Cr                                       | 20.00  | Cu | 1.5 |
| Mo                                       | 4.50   | Sn | 2.0 |
| Mn                                       | 1.25   | Ga | 2.0 |
| Proportional Limit (psi)                 | 37,000 |    |     |
| 0.2% Yield Strength (psi)                | 47,400 |    |     |
| Ultimate Tensile Strength (psi)          | 73,600 |    |     |
| Elongation (%)                           | 11     |    |     |
| Rockwell "B" Hardness                    | 86     |    |     |

25

## EXAMPLE VI

An alloy having the composition listed below was prepared in accordance with the procedure described in the Example I, and test specimens were prepared by investment casting of the alloy to obtain defect-free cast alloy shapes having the physical characteristics also listed below.

| Composition (% by weight) and properties |        |    |     |
|------------------------------------------|--------|----|-----|
| Ni                                       | 66.25  | Si | 2.5 |
| Cr                                       | 20.00  | Cu | 1.5 |
| Mo                                       | 4.50   | Sn | 1.0 |
| Mn                                       | 1.25   | Ga | 3.0 |
| Proportional Limit (psi)                 | 37,200 |    |     |
| 0.2% Yield Strength (psi)                | 46,700 |    |     |
| Ultimate Tensile Strength (psi)          | 68,700 |    |     |
| Elongation (%)                           | 9      |    |     |
| Rockwell "B" Hardness                    | 86     |    |     |

35

## EXAMPLE VII

An alloy having the composition listed below was prepared in accordance with the procedure described in the Example I, and test specimens were prepared by investment casting of the alloy to obtain defect-free cast alloy shapes having the physical characteristics also listed below.

| Composition (% by weight) and properties |      |    |     |
|------------------------------------------|------|----|-----|
| Ni                                       | 75.5 | Cu | 1.5 |
| Cr                                       | 15.0 |    |     |

65

-Continued

| Composition (% by weight) and properties |        |    |     |
|------------------------------------------|--------|----|-----|
| Mn                                       | 0.5    | Ga | 7.5 |
| Proportional Limit (psi)                 | 35,000 |    |     |
| 0.2% Yield Strength (psi)                | 42,500 |    |     |
| Ultimate Tensile Strength (psi)          | 69,000 |    |     |
| Elongation (%)                           | 16     |    |     |
| Rockwell "B" Hardness                    | 72     |    |     |

10

## EXAMPLE VIII

The foregoing alloy compositions were modified by the inclusion of up to 10 percent by weight molybdenum, up to 9 percent by weight of tin and 7.5 percent by weight of gallium, up to 5 percent by weight copper, up to 4.0 percent by weight silicon, up to 2.0 percent by weight aluminum and up to 5 percent by weight cobalt. All possessed the improved physical properties characteristic of the alloy composition of the invention.

We claim:

1. A corrosion resistant hot workable and hardenable precision casting alloy consisting essentially, by weight:

|            |              |
|------------|--------------|
| Nickel     | at least 60% |
| Chromium   | 10 - 25%     |
| Molybdenum | 0 - 10%      |
| Manganese  | 0.50 - 1.50  |
| Tin        | 0 - 6.5      |
| Gallium    | 1.0 - 7.5    |
| Copper     | 0 - 5.0      |
| Silicon    | 0 - 4.0      |
| Aluminum   | 0 - 2.0      |
| Cobalt     | 0 - 5.0      |
| Carbon     | 0 - 0.2      |

the combined total amount of tin and gallium not exceeding 7.5.

2. The corrosion resistant alloy according to claim 1 consisting essentially by weight:

|            |                  |
|------------|------------------|
| Nickel     | 68.25%           |
| Chromium   | 20.0%            |
| Molybdenum | 4.5%             |
| Manganese  | 1.25%            |
| Gallium    | 2.0%             |
| Copper     | 1.5%             |
| Silicon    | 2.5%             |
| Carbon     | Less than 0.01%. |

3. The corrosion resistant alloy according to claim 1 consisting essentially, by weight:

|           |                  |
|-----------|------------------|
| Nickel    | 75.5%            |
| Chromium  | 15.0%            |
| Manganese | 0.5%             |
| Gallium   | 7.5%             |
| Copper    | 1.5%             |
| Carbon    | less than 0.01%. |

4. The corrosion resistant alloy according to claim 1 consisting essentially, by weight:

|            |                  |
|------------|------------------|
| Nickel     | 66.25%           |
| Chromium   | 20.0%            |
| Molybdenum | 4.5%             |
| Manganese  | 1.25%            |
| Tin        | 3.0%             |
| Gallium    | 1.0%             |
| Copper     | 1.5%             |
| Silicon    | 2.5%             |
| Carbon     | less than 0.01%. |

**5. The corrosion resistant alloy according to claim 1  
consisting essentially, by weight:**

|            |                  |
|------------|------------------|
| Nickel     | 68.25%           |
| Chromium   | 20.0%            |
| Molybdenum | 4.5%             |
| Manganese  | 1.25%            |
| Tin        | 1.0%             |
| Gallium    | 1.0%             |
| Copper     | 1.5%             |
| Silicon    | 2.5%             |
| Carbon     | less than 0.01%. |

5

**6. The corrosion resistant alloy according to claim 1  
consisting essentially, by weight:**

|            |        |
|------------|--------|
| Nickel     | 66.25% |
| Chromium   | 20.0%  |
| Molybdenum | 4.5%   |

10

|            |        |
|------------|--------|
| Nickel     | 66.25% |
| Chromium   | 20.0%  |
| Molybdenum | 4.5%   |

15

|            |        |
|------------|--------|
| Nickel     | 66.25% |
| Chromium   | 20.0%  |
| Molybdenum | 4.5%   |

20

|            |        |
|------------|--------|
| Nickel     | 66.25% |
| Chromium   | 20.0%  |
| Molybdenum | 4.5%   |

25

|            |        |
|------------|--------|
| Nickel     | 66.25% |
| Chromium   | 20.0%  |
| Molybdenum | 4.5%   |

30

|            |        |
|------------|--------|
| Nickel     | 66.25% |
| Chromium   | 20.0%  |
| Molybdenum | 4.5%   |

35

|            |        |
|------------|--------|
| Nickel     | 66.25% |
| Chromium   | 20.0%  |
| Molybdenum | 4.5%   |

40

|            |        |
|------------|--------|
| Nickel     | 66.25% |
| Chromium   | 20.0%  |
| Molybdenum | 4.5%   |

45

|            |        |
|------------|--------|
| Nickel     | 66.25% |
| Chromium   | 20.0%  |
| Molybdenum | 4.5%   |

50

|            |        |
|------------|--------|
| Nickel     | 66.25% |
| Chromium   | 20.0%  |
| Molybdenum | 4.5%   |

55

|            |        |
|------------|--------|
| Nickel     | 66.25% |
| Chromium   | 20.0%  |
| Molybdenum | 4.5%   |

60

|            |        |
|------------|--------|
| Nickel     | 66.25% |
| Chromium   | 20.0%  |
| Molybdenum | 4.5%   |

65

|           |                  |
|-----------|------------------|
| Manganese | 1.25%            |
| Tin       | 2.0%             |
| Gallium   | 2.0%             |
| Copper    | 1.5%             |
| Silicon   | 2.5%             |
| Carbon    | less than 0.01%. |

8

**7. The corrosion resistant alloy according to claim 1  
consisting essentially, by weight:**

|            |                  |
|------------|------------------|
| Nickel     | 66.25%           |
| Chromium   | 20.0%            |
| Molybdenum | 4.5%             |
| Manganese  | 1.25%            |
| Tin        | 1.0%             |
| Gallium    | 3.0%             |
| Copper     | 1.5%             |
| Silicon    | 2.5%             |
| Carbon     | less than 0.01%. |

\* \* \* \* \*

25

30

35

40

45

50

55

60

65